

# UNITED STATES PATENT OFFICE.

JESSE S. EGGLESTON, OF AUBURN, NEW YORK, AND JOHN RICH, OF BURLINGTON, VERMONT.

## IMPROVEMENT IN LUBRICATING COMPOUNDS.

Specification forming part of Letters Patent No. 154,130, dated August 18, 1874; application filed June 9, 1874.

*To all whom it may concern:*

Be it known that we, JESSE S. EGGLESTON and JOHN RICH, respectively of Auburn and Burlington, in the counties of Cayuga and Chittenden and States of New York and Vermont, have invented certain new and useful Improvements in Lubricating Compound; and we do hereby declare the following to be a full, clear, and exact description of the invention, such as will enable others skilled in the art to which it pertains to make and use it.

Our invention relates to a new and improved lubricating compound, possessing many advantages over the lubricating oils and compounds in ordinary use, both in cheapness and durability, and which will not turn rancid or decompose and corrode the iron or other metal with which it comes in contact, as other lubricating compounds and oils are apt to do. Our compound also possesses the property of mingling or mixing with steam, and thus more effectually accomplishing its work when employed to lubricate steam machinery. Our invention is designed particularly to be used as a lubricant for steam-cylinders and steam-chests and the other working parts of steam-engines, in which the lubricant is liable to come in contact with the steam.

Our invention consists of a compound of borax, oil, and water. We use either animal, vegetable, or mineral oil, in the following proportions, viz.: Borax, say, five pounds; West Virginia or other oil, thirty gallons; water, say, ten gallons. These ingredients we

mix, preferably by the aid of heat; but under some circumstances they may be combined in a cold state, although it takes longer to effect a thorough chemical union of the different ingredients when combined without the aid of heat. We agitate the mass, by stirring or otherwise, after mixing, until the mass assumes a homogeneous unctuous form, when it is ready for use. The compound we apply in the same manner as the ordinary lubricants, by means of the ordinary oil-cups attached to the steam-chests and cylinders of engines, and, as it is liquid, it finds its way to the working parts of the engine in the same manner as oil.

We do not limit ourselves to the exact proportions of ingredients as above set forth, because the proportions may be varied without departing from the nature of the invention.

Having described our invention, what we claim, and desire to secure by Letters Patent, is—

The within-described compound, consisting of borax, oil, and water, in about the proportions of five pounds of borax, thirty gallons of oil, and ten gallons of water, substantially as and for the purpose described.

In testimony that we claim the foregoing, we have hereunto set our hands this 1st day of June, 1874.

JESSE SCOTT EGGLESTON.  
JOHN RICH.

Witnesses:

JOEL B. THOMAS,  
A. J. HOWARD.